

Nov. 16, 1937.

E. FREYSSINET

2,099,265

PROCESS FOR THE MANUFACTURE OF MOLDED PIECES FROM MORTARS OR CONCRETE

Filed Feb. 5, 1934

4 Sheets-Sheet 1



INVENTOR  
Eugene Freyssinet,  
By Paton, Coit, Moore & Lindley  
Hanns.

Nov. 16, 1937.

E. FREYSSINET

2,099,265

PROCESS FOR THE MANUFACTURE OF MOLDED PIECES FROM MORTARS OR CONCRETE

Filed Feb. 5, 1934

4 Sheets-Sheet 2



INVENTOR

*Eugene Freyssinet,  
By Paton, Coit, Moore & Lindley.*

ATTYS.

Nov. 16, 1937.

E. FREYSSINET

**2,099,265**

## PROCESS FOR THE MANUFACTURE OF MOLDED PIECES FROM MORTARS OR CONCRETE

Filed Feb. 5, 1934

4 Sheets-Sheet 3



*INVENTOR*

Eugene. Dryasinae.  
By Watson, Capt. Moore & Grindell.  
1875.

Nov. 16, 1937.

E. FREYSSINET

**2,099,265**

## PROCESS FOR THE MANUFACTURE OF MOLDED PIECES FROM MORTARS OR CONCRETE

Filed Feb. 5, 1934

4 Sheets-Sheet 4



Fig. 11c



Fig. 10a



Fig. 10

INVENTOR

Eugene Drygasinski

By Nation, Coit, Moore & Lindell

ATTYS.

## UNITED STATES PATENT OFFICE

2,099,265

PROCESS FOR THE MANUFACTURE OF  
MOLDED PIECES FROM MORTAR OR CON-  
CRETE

Eugène Freyssinet, Neuilly-sur-Seine, France

Application February 5, 1934, Serial No. 709,877  
In France February 9, 1933

## 4 Claims. (Cl. 25—155)

The present invention relates to methods and apparatus for the manufacture of molded pieces or bodies from mortars or concretes that are moist and even contain an excess of water, in which methods these concretes or mortars are subjected to the action of a vibration and a compression, in order to drive out the excess of water and to rapidly produce an article having the maximum hardness that is possible.

5 I have found out that vibration causes a settling of the concrete at the lower part of the mold while the excess of water accumulates in the upper part which thus becomes filled with soft concrete. Under these conditions, compression produces de-  
10 formations of the concrete that vary according to the level in the mold and the articles thus obtained may be utterly spoiled.

On the other hand it is important, in order to keep the deformable or expandable organs serving 20 to compress the concrete in good working order, and also in order to obtain regularly and accurately shaped articles, that the deformations of these organs should be small, corresponding for instance to a small reduction of thickness of the 25 concrete in the mold.

A first feature of the method according to the present invention consists in performing the treatment in two steps, one that consists in simultaneously vibrating and compressing the concrete, 30 the compression being relatively weak, in order that it may not prevent the relative displacement of the concrete particles under the effect of the vibration, and the second step consisting in strongly compressing the concrete which has been 35 rendered firm and compact by the first step of the treatment.

Another feature of my invention consists in connecting with the portions of the mold in which the concrete has a tendency to become too 40 fluid complementary chambers which are filled with concrete at the same time as the mold. These chambers are so arranged that the portions of the mold that have a tendency to become exaggeratedly fluid in the course of the vibrating treatment are transferred into said chambers so that the mold finally contains only concrete having a 45 homogeneous structure.

I thus obtain that the mold is exactly filled with 50 concrete. The complementary chambers can be separated without difficulty by producing a relative sliding displacement of the complementary chambers and of the mold along their joining surface, which must be either a plane surface of a 55 surface of revolution. The complementary chambers may be provided along these surfaces with

organs acting as knives or plugs making it possible to obtain, after removal of these complementary chambers, very clean and regular limiting surfaces for the concrete, without any risk of concrete dropping from the complementary 5 chambers when they are removed.

The combination of these two features makes it possible to obtain a perfect result from the point of view of both the compactness and the homogeneity of the concrete that is obtained. These 10 two features are closely interrelated because the compression of the concrete in the mold, during the vibrating treatment, can be advantageously obtained under the effect of the pressure resulting from the height of concrete filling the complementary 15 chambers, provided that these chambers are suitably disposed above the mold.

Other means for creating the desired pressure in the mass of concrete in the mold may consist of one or several pistons adapted to compress the 20 concrete in the molds, these pistons being either partly immersed directly in the concrete or disposed inside a corresponding cylinder. They may be made in any suitable manner, consisting for instance of rods or bundles of rods, made of steel, 25 wood or any other material, bearing on the concrete, slight spaces being reserved between them and the cylinder for the escape of the excess of water, air, etc. These pistons may act either by their own weight or be subjected to other loads. 30 I may also place at a suitable point, for instance in a complementary chamber, an expandable element, such as a rubber bag which will be inflated by means of water or air. Finally, I may also make use of a concrete pump for filling the mold 35 and subject the concrete therein to the desired pressure.

I must further provide in the mold apertures adapted to prevent the concrete, including the fine particles thereof, from escaping from the 40 mold, while allowing water and air to be driven out therefrom, these apertures being located sufficiently below the free surface of the concrete for causing the concrete in the vicinity of said apertures to undergo a sufficient pressure for compacting 45 the solid elements thereof while facilitating the escape of air and water in excess.

In order to carry out the method above explained it is particularly advantageous to make use, for constituting the complementary chamber that serves both to subject the concrete in the mold to the required pressure during the vibrating treatment and to receive the portions of the concrete that are too fluid, of a hopper of sufficient height, located above the mold, with 55

which it communicates. This hopper will further serve to the filling of the mold and to vibrate the concrete in the mold due to the vibrations of its walls and of the walls of the mold which are 5 temporarily rigidly connected with said hopper.

My invention further includes a particular application of the method above set forth to the manufacture of articles of any shape and size by successive elements perfectly connected to one 10 another. For this purpose, I provide, on the one hand, temporary connecting organs between each finished element and the mold that is to serve to the manufacture of the next element, these organs being capable of withstanding the stresses 15 which, due to the vibrating and compressing treatments, will tend to separate the concrete already hardened from the next element to be fixed thereto; and on the other hand, permanent connecting organs between the successive elements. The temporary connecting organs between the concrete and the mold can be obtained by providing in the outer portions of the mold 20 an end element the walls of which are in contact with the concrete are corrugated or rough, so as to adhere strongly thereto, this element being left in position until the concrete is hardened and is sufficiently strong for resisting the efforts to which it will be subjected in the course of the following operations. The 25 connection between the concrete and the mold may also result from holes provided in the concrete and adapted to cooperate with bolts or other known connecting means. The connection may also be insured by means of organs 30 sealed in the concrete, such as inwardly threaded rods, bolts or fastening rings. The permanent connecting organs may consist of reinforcements 35 projecting from the concrete or of recesses provided in the latter and intended to be molded with the following element. For instance the inner expandable elements are provided with one or several projections at their end located on the side where the next element is to be added, said 40 projections being of suitable shape for providing in the molded concrete a recess of corresponding shape in which will be inserted the reinforcements and the concrete through which an element is rigidly connected with the next element. Special expandable elements can be substituted 45 for one or several of these projections.

50 Other features of my invention will result from the following detailed description thereof.

Preferred embodiments of the present invention will be hereinafter described with reference to the accompanying drawings, given merely by way of example, and in which:

55 Figs. 1 and 2 are diagrammatical views illustrating means for obtaining a moderate compression of the concrete during the vibrating treatment;

Fig. 3 shows, partly in sectional view and partly in diagrammatic perspective view, a device for carrying out the process according to my invention which includes a hopper for filling the 60 mold, which also acts as means for compressing the concrete in the mold, complementary chamber, and vibrating means;

Fig. 4 shows how the mold can be closed after being filled with concrete;

70 Figs. 4a and 4b a cross section on the line 4a—4a of Fig. 4b and a side view respectively of another device for closing the mold;

Fig. 5 shows a vibrating device disposed on the inside of the core;

75 Fig. 6 is a cross section of an expandable organ

consisting of a plurality of staves subjected to the action of an elastic mandrel;

Figs. 7, 8 and 9 show details of this expandable organ;

Fig. 10 is a sectional view of a mold provided 5 with an expandable organ of this kind;

Figs. 10a and 10b are a cross section and a longitudinal section respectively of a device for closing the ends of the elastic mandrel;

Fig. 11 is a diagrammatical view of another 10 embodiment of the device for closing the end of the mandrel;

Fig. 11c shows a device for operating the cores;

Figs. 12 to 15 are diagrammatical views illustrating other embodiments of the invention; 15

Fig. 16 is a vertical sectional view illustrating the manufacture of concrete piles or stakes by successive elements;

Fig. 17 is a diagrammatical view illustrating the manufacture of a large size building element, 20 for instance a bridge arch.

Figs. 1 and 2 show a mold wall 1 having a series of points *a*, *b*, *c*, *d*—*h* located at a higher level where there have been provided different devices for obtaining a moderate compression of 25 the concrete 1\* in the mold and for simultaneously allowing water and air to escape; 2 is a plug consisting of a plurality of wooden plates which do not fit exactly with each other, said plug being maintained by a plate 3 and a screw 4; 5 is another plug made of a filtrating material, such as 30 felt, horse-hair, etc., maintained in position by a removable plate 6, fixed by means of screws and nuts 7; 8 is an autoclave joint which is not watertight, which is kept in position during the filling 35 of the mold by an elastic organ 9; 10 is an external closure plate maintained by a screw 11; 12 is a plunger piston acting in a cylinder 13 which may be used as a filling hopper and as a complementary chamber, this piston being actuated by a hydraulic jack 14 so as to compress the concrete in the mold; 15 is a floater reducing to a minimum the volume of concrete contained in a complementary chamber 16; 17 is a piston consisting of a plurality of rods or blades resting on 40 the surface of the concrete and allowing water to leak out through the interstices between them; 18 is a rubber bag inflated through a pipe 19 and acting in a chamber 20 closed by joints 21, 22 that are not watertight.

50 In Fig. 3, the mold consists of two mold elements 23, 24 assembled along their lower edge through a longitudinal autoclave joint 25 forming a double joint for the escape of water and also through jaws 26 coacting with a yielding organ 27, for instance 55 made of wood and provided with holes, so as to form a flexible joint allowing water, and even concrete, to leak out.

Between the upper edges 28, which are thick, rigid and horizontally disposed, of this mold, I 60 provide two steel lips 29 having a rubber coating which projects inwardly at 30. These lips prolong the walls 31 of a sheet iron hopper supported by members 32 resting on rubber parts 33. This hopper is closed, at its front and rear ends, 65 by metal plates 34 connected together by a rubber membrane 35, or any other organ permitting a displacement of walls 31 with respect to each other. These walls 31 can be pushed toward each other, so as to close the passage between projections 30, by operating hydraulic jacks 36 acting through suitable levers on rubber pads 37 carried by the walls of the hopper. On the contrary these walls 31 can be moved away from each other so as to open this passage between pro- 70 75

5 jects 30 (when the mold is being filled) by discharging the working water from these jacks. Other hydraulic jacks 38, distributed along the hopper and bearing against the edges 28 of the mold, can strongly apply these edges against the lips 29 of the hopper.

10 Each element of the hopper is connected with bearings 39 distributed over its length and in which are journalled shafts 40a, 40b carrying, close to said bearings, eccentric masses 41a, 41b disposed in the same plane for each of said shafts. Bearings 39, shafts 40a and 40b, and also masses 41a, 41b are symmetrically disposed to the vertical median plane of the hopper. Shafts 40a, 15 40b are connected together by a system of gears, for instance bevel gears 42, causing them to turn in opposite directions and with the same speed of revolution.

20 The coupling of gear wheels 42, which must not move together with the hopper, with shafts 40a, 40b, each connected to one half of the hopper, is ensured by means of elastic organs sufficiently rigid for maintaining a sufficient synchronization of the movements of the shafts. In 25 the embodiment of Fig. 3, these coupling organs include a fork-shaped piece 43 the ends of which are surrounded by rubber cylinders 44 engaging in corresponding recesses 45 rigidly connected to the portion of the shaft driven by the bevel gear 30 wheels.

25 In the case of hoppers and of molds of great length, similar organs can be interposed between several portions of shafts 40a and 40b, in order to facilitate the taking to pieces.

30 When the gear wheels are actuated by a motor 46, the bearings 39, the walls 31 of the hopper, and also the lips 29 at the lower part thereof are given symmetrical vibratory movements, the amplitude of which depends on the 35 ratio of the masses depending on the hopper and the product of the eccentric masses and of their eccentricity.

35 On the other hand, the intensity of the vibratory accelerations increases proportionally with 40 the square of the speed of revolution.

45 It is therefore to vary at will the amplitude of the movements of the mold and the energy of the vibratory movement independently of each other, by varying the eccentric masses and the speed of 50 revolution of the shafts that carry said masses. This vibration is transmitted to the mold through lips 29 when pressure is applied thereto through jacks 38. The passage between said lips is opened and closed several thousands of times per minute 55 (the width of this passage being for instance of about 1 millimeter, although it can be considerably greater or smaller) and the walls of the mold and the system consisting of wood piece 27 and jaws 26 are elastically deformed.

60 The value of the alternating accelerations is about ten times the acceleration of gravity; but this is merely an indication and these alternating accelerations might be considerably greater or smaller.

65 Concrete in the plastic state and even in a relatively firm state, when poured into the hopper at any point thereof during the vibratory treatment, assumes the appearance of a liquid, having a horizontal level surface, so that the 70 mold is perfectly filled, even in its smallest interstices, and more particularly in the vicinity of reinforcements such as 113, which have been disposed in advance in the mold.

75 Furthermore, if the amount of concrete introduced into the hopper is greater than that neces-

sary for filling the mold, so that, once said mold is full, a certain amount of concrete remains in the hoppers, up to a height  $h$  the concrete in the mold is compressed, during the whole vibrating treatment, with a pressure the value of which depends on  $h$ . 5

Finally, the hopper plays, during this vibratory treatment, the part of a complementary chamber as above explained, the excess of water in the concrete of the mold accumulating in the upper part 10 of the concrete in the hopper, while the vibratory treatment causes the solid particles of said concrete in the hopper to pass into the mold which is thus filled with homogeneous concrete at the end of the vibrating treatment. This treatment 15 lasts for some minutes, after which motor 46 is stopped and water is discharged from the hydraulic jacks 38, jacks 38 being kept under pressure. The mold, now exactly full with compact concrete can then be separated from the hopper 20 by moving in a downward direction support 47, for instance by means of jacks 48. The orifice between the upper edges 28 of the mold is then stopped by means of a plate of wood, metal or both of these materials, 48a, which can be maintained in position through any suitable known means, for instance by means of jaws 26a (Fig. 4) or by straps 110 (Figs. 4a and 4b) applied by means of tightening elements the tension of which can be adjusted by means of a screw 30 engaging in element 112.

25 When the mold is thus closed the concrete therein can be subjected to the second part of the process according to the present invention which consists in strongly compressing it by 35 means of an expandable mandrel disposed inside the mold and made, for instance, as it will be hereinafter described.

30 Vibration can be produced through many other means. In some cases, it will be advisable to 40 produce it by the rotation of eccentric masses such as 50 (Fig. 5) disposed on the inside of the mold itself, for instance in the expandable central core 51, said masses being carried by shaft 52 the bearings of which are rigidly supported by said 45 core. Instead of being transmitted to the mold through the hopper, as in the embodiment of Fig. 3, the vibrations can also be directly transmitted to the walls of the mold, by connecting 50 said walls with the bearings of the shaft carrying the eccentric revolving masses.

55 The expandable organs serving to carry out the second part of the process according to the present invention and on which the concrete is molded during the first part of the process must have 60 a rigid and definite shape so as to permit of obtaining correct molded articles of uniform thickness, even during this first step of the process.

65 These expandable organs are of two kinds. In the first kind, an example of which is 65 shown in Figs. 3 to 5 inclusive, and more specifically in Fig. 4a, there is provided a rigid core 51 of wood or metal of the desired shape covered by an elastic bag 53, for instance of india-rubber, which will be generally strengthened by fabrics or cables such as 53a in at least one direction, owing to the small deformation to which these organs are subjected. A fluid is introduced at the desired time between the core and the bag through pipes such as 54.

70 In the second kind, an example of which is shown in Figs. 6 to 10, the expandable organ consists of a system of staves such as 55 made of a strong material, such as steel, bakelite, wood, either impregnated or natural, disposed around 75

75

an india-rubber expandible envelope 53, either free or mounted on a rigid mandrel 51, as in the preceding case. These staves are suitably shaped so as to constitute, when they are assembled together, a well determined structure, against which concrete can be molded in an accurate manner. If the elastic envelope 53 is inflated by means of a fluid under pressure, the staves are pushed apart, thus compressing the concrete and 10 opening between them very fine interstices for the outflow of water, the width of these interstices increasing as the concrete is being more compressed, so that the outflow of water from the concrete takes place under the best conditions, this outflow being eventually facilitated by providing grooves in the sides of the staves. In order to avoid that the elastic envelope may engage into the interstices between the staves, the latter will be provided with pieces such as 56 (Figs. 7 and 8) 15 made of metal, wood, stronger india-rubber, or a fabric of suitable shape, normally folded for instance so as to permit the expansion of india-rubber while preventing it from penetrating into the interstices between the staves. The same result can be obtained by means of wires 57 disposed very obliquely with respect to the generatrices of the cylinder (Fig. 9).

In both of the embodiments just above described, the elastic bag or envelope may consist 30 of various materials of elastic structure arranged in various manners. It may for instance consist of a double rubber wall forming a closed flat bag which may be inflated through an aperture such as the valve of the inner tube of a pneumatic 35 tire. It may also consist of a fluidtight internal mandrel with an external rubber envelope joined to said mandrel through any suitable means such as: an autoclave joint analogous to a cup-leather packer, or an elastic envelope inserted between 40 the core and an external envelope and inflated at a pressure higher than that existing between the envelope and the mandrel.

This last arrangement will be more specifically described with reference to Figs. 10a and 10b, 45 which correspond to the type of mold and of elastic mandrel shown in detail in Figs. 4a and 4b. A plate 117, made of such a size that it may cover the extreme edges of the mold portions 23 and 24, is provided in its middle part with a 50 hole accommodating core 51 and elastic envelope 53. Around this hole there is fixed a gutter shaped hollow part 118 in which is mounted an elastic tube 119 of the kind of the inner tube of a pneumatic tire, and adjusting elements such as 120 and 121, which may be made of rubber, strengthened in a direction parallel to the axis of the mold. If a fluid under a suitable pressure is introduced into this tube 119, it strongly applies elastic envelope 53 against core 51. The 55 elements 120 and 121 make it possible to vary to a substantial degree the size of the cores that can be utilized with the device. The whole must be maintained against the end of the mold in any suitable manner for resisting the pressures.

I have shown in Fig. 11 a second example in 60 which an elastic envelope 53 is disposed around a rigid core 51, staves 55 being arranged around said envelope. The elastic envelope 53 is maintained at the ends of the core by an end plate 58 which bears against shoulders provided in staves 55. This end plate 58 and the plate located at the other end of the mold could also be maintained by metal rods, wires, or cables passing through holes or grooves provided in the 65 staves (wires 70, Fig. 16, holes 71, Fig. 6). They

could also be dispensed with by giving a suitable shape to the end of the elastic envelope, which is supposed to be reinforced in the longitudinal direction by means of inextensible wires, of fibre, textile material or metal. 5

The deformation of the concrete that results from its being compressed increases the inner volume, thus creating a play which will permit, as a rule, to remove the expandible organ. If the core is of elongated shape and horizontally 10 disposed, its removal by causing it to slide out from the fresh concrete article may be somewhat difficult. This difficulty can be obviated by supporting it at a single point of its larger end by means of a carriage such as that shown in Fig. 15 11c. This carriage 130 can be engaged under the mold so that the center of gravity 131 of the core may be located between the ends 132, 133 of the carriage. The latter comprises longitudinal wheels 134 and transversal wheels 135, which 20 can be brought into inoperative positions by any known device such as that including articulations 136 and levers 137. Wheels 134 can be adjusted at any desired height by means of springs 138 balancing the weight of the system. The core 25 is provided with a part 139 pivoted about an axis 140 to the frame of the carriage. A lever 141 having an arcuate portion 142 acting as a pulley having its center on axis 140 is also pivoted to the frame about said axis or one located very 30 close to it. This lever 141 can be actuated through a mechanism 143 including for instance a screw.

Cables 144 adapted to slide in tubes 145 are secured to points 146 of the core. These cables 35 pass over portion 142 and are fixed to lever 141 at 147.

An action on these cables produces reactions converging at 140, the vertical components of which at points 146 balance the weight of the 40 core. Points 146 may be so determined that the elastic deformation of the core when it is lifted by acting thereon through 143, produces no other deformation than a longitudinal compression. The core is thus supported under conditions such 45 that its handling becomes very easy.

I may also facilitate the removal of the core by making it of several parts one of which, in the shape of a wedge, will permit the removal of the others. In the case of mandrels consisting of an assembly of staves, it will be advantageous to insert between two staves, a steel blade such as 59, having parallel or slightly divergent faces (diverging toward the inside of the mold), which will be easily driven in toward the center, 55 once the pressure exerted through the elastic envelope is removed.

By means of one or the other of the expandible organs above described, or by their combination, it will be possible to obtain recesses of 60 any desired shape, either simple or multiple, either cylindrical or of complex shape, provided with grooves if the expandible organs are located at the periphery of the mold, etc. It will be also possible to make use of very flat expandible elements disposed between the wall of the mold and the concrete, such as shown at 67a in Fig. 15. In Fig. 10, an auxiliary expandible organ 72 disposed in the annular mass of concrete permits of obtaining a conduit therethrough and a second expandible organ 73, provided at the periphery of the concrete permits of obtaining a groove. 65

The reduction of the volume of the mold can also be obtained in other manners without departing from the principle of the present inven- 70 75

tion. For instance, as shown in Fig. 12, the mold can be made of two portions 60, 61, part 60 being stationary and part 61 being movable by means of a jack 62, or of a rubber bag, or through any other means. I may also, as shown in Fig. 13, associate together two molds 63, 64 and compress the concrete between these molds by means of plates 65 between which are mounted jacks 66, rubber bags, or equivalent means. In Figs. 10, 14 and 15, the mold is divided into several portions by several expandible organs 67.

The pressure applied during the second part of the process may vary between some hundreds of grammes per square centimeter and some hundreds of kilogrammes per square centimeter. The only limits that exist are imposed by the necessity of making sufficiently strong molds. The results that are obtained are so much the better as the pressure is higher. This is why it is important to make molds as strong as possible, by providing them with reinforcing members as in the embodiment shown in Figs. 4a and 4b, or by giving their section a suitable shape, for instance a circular shape, the parts being assembled by means of screw jaws 26 acting tangentially to the curve of tensions in the metal of the mold (Fig. 10). However, it is possible to produce with these molds articles of any desired section by distributing at the proper places cores of suitable shape. It is also possible to utilize molds formed by walls of any shape whatever, adapted to the special use that is considered, said walls being connected together, and particularly through the concrete, by bolts extending through tubes of concrete prepared in advance and which are left in the mass or surrounded by tubes of rubber or any other plastic material permitting their removal and an example of which will be described with reference to Fig. 17.

As a rule, no vibration will be effected during the final compression because vibration may, in this case, produce a settling of the concrete around the lower portions of the core, so that the increase of volume resulting from the compression will take place only at the upper part of the latter, this involving an irregular form of the finished article, difficulties in the removal from the mold, and frequently the injuring of the expandible organs.

In special cases in which such drawbacks are not to be feared, it is however possible to maintain the vibratory treatment during the second part of the process, because it will facilitate the outflow of the excess of water, which, due to the stopping of the vibratory treatment, becomes more difficult. In such cases, the second step of the process is a mere continuation of the first one, characterized by the use of a higher pressure.

Starting from concretes that are as fluid as it is desired for obtaining a good filling of the mold (which may be of complicated shape or encumbered with reinforcements) it is possible, with the process according to my invention to obtain in some minutes the consistency of very hard macadams, the articles thus obtained being much stronger than concrete articles molded in the dry state and compressed in a press. Furthermore, the concrete is very adhesive to its reinforcements. This consistency permits in any case immediately to remove the concrete piece from either the inner or the outer mold and very often from both at the same time, even when the pieces are of complicated shape, or very thin, or of very large size.

The hardening of concrete treated by the process above described is extraordinarily rapid. In the case of pressures averaging 20 kilogrammes per square centimeter applied to concretes sufficiently rich in very fine elements, I obtain, with good aluminous cements, at an average temperature of 15° C.:

|                                                   | Kg/cm <sup>2</sup> | 15 |
|---------------------------------------------------|--------------------|----|
| 3 hours after the tempering a resistance of from  | 150 to 300         | 10 |
| 8 hours after the tempering a resistance of from  | 400 to 800         |    |
| 18 hours after the tempering a resistance of from | 500 to 1000        |    |

With Portland cements equivalent resistances are obtained after periods of times above four or five times longer, at the same average temperature of 15° C.

By heating progressively from 15 to 80° C. or 90° C. in a saturated atmosphere and under conditions capable of avoiding dehydrating of the concrete, it is possible to shorten the times of hardening for Portland cements down to the values above indicated for aluminous cements. In this case, there is a difficulty that results from the heat of setting of the cements which tends, by raising their temperature above that of the heating medium, to dehydrate them the more rapidly as they contain but just the amount of water that is necessary for their setting, which prevents their hardening. A concrete at a temperature of 85° becomes quickly dehydrated in air at a temperature of 80°, even saturated with water vapor. This drawback can be obviated by progressively increasing the temperature of the medium so that it is always hotter than the concrete, until a sufficient hardening is obtained. For this purpose I send, for instance, water vapor around and into the concrete article to be heated, placed in a heat insulated envelope, consisting eventually of the mold itself, with an adjustable rate of flow so as to obtain the desired law of variation.

I have found that, in order to further increase the rapidity of hardening, it suffices to let a certain time elapse between the end of the first step of the process and the beginning of the second, this time being sufficient for causing the setting to have started when the high pressures applied during the second step of the process are brought into play. I may also, for the same purpose, prolong the first step of the process until the setting of the concrete has started.

I may further indicate, as one of the results of the quick hardening of the concrete and of the regularity of molding which result from the process according to the present invention, the possibility of manufacturing objects of unlimited length and width, and of any desired shape, by making it in successive portions perfectly well connected and secured to one another.

I will describe two examples of such a manufacture. The first example will be explained with reference to Fig. 16 of the accompanying drawings which illustrates a method of manufacturing piles the successive portions of which are molded vertically after sinking of the preceding portions.

The outer portions of the mold are provided with an end element 81 whose wall in contact with the concrete is corrugated or rough so as to adhere strongly thereto. In Fig. 16 the end element 81 is in position at the upper part of a pile portion A previously manufactured and sunk.

The question is now to make the following portion B. I place over end element 81 a cylindrical shell 82 and another end element 81<sup>a</sup> similar to the first one, these parts being assembled through rods 83 tightened by means of nuts in lugs 83<sup>a</sup> provided on the end elements.

In the mold thus formed I place an expandible cylindrical organ consisting of a rigid core 51, a rubber envelope 53 and staves 55, the core and 10 the staves being maintained in position by means of wires or rods 70 extending through grooves provided in the staves and connecting the end plates 58 together. This core further comprises at its upper end an annular projection 84 reducing at this place the interval between the core and the mold. In the manufacture of portion A of the pile, this projection 84 has produced an annular recess which is visible at 84<sup>a</sup> and which will serve to connect portions A and 20 B together. The connecting reinforcements 85, distributed in the concrete of portion A project into this recess.

I may also provide other cores such as those shown in Fig. 10 at 72 and 73, the last mentioned cores being or not provided with projections.

These projections of the expandible organs can be replaced by special expandible cores of suitable length adapted to reserve sufficient recesses for a good sealing of the connecting reinforcements.

I dispose, above the interval between the core and the mold, an annular hopper 85 and I pour thereinto an amount of concrete sufficient for 35 filling the mold and the hopper up to a height *h*. The concrete is vibrated in the course of this filling, for instance by rotating, in bearings rigidly connected with the mold, shafts carrying eccentric masses, or in any other way. This 40 vibratory treatment is prolonged for a sufficiently long time, once the mold is full, for driving out the excess of water. The hopper then plays the part of a complementary chamber and of an organ for moderately compressing the concrete 45 in the mold, owing to the amount of concrete that it contains. After eliminating the air and the water in excess in the mold and obtaining therein a compact and homogeneous concrete, the hopper is removed and it is replaced by a 50 closure plate 87 (shown in dotted lines in the drawings) connected to the end element 81 by rods 88 fixed in the lower lugs 83<sup>a</sup>. Fluid under pressure is then introduced into the elastic envelope through pipe 89 so that the excess of 55 water of the concrete flows out through the staves. This compression, which pushes the concrete toward the outside, has for its effect to weld the lower part of portion B with the upper part of portion A previously manufactured in 60 the annular recess 84<sup>a</sup> provided at the upper part of the last mentioned portion of the article to be obtained. The pressure is removed, the elastic mandrel, the staves, then the portions of the mold and finally end element 81 are removed. 65 I leave in position the end element 81<sup>a</sup> which reinforces the end of portion B against the stresses that it may have to withstand in the course of the following operations, for instance for sinking it. The following portion of the 70 pile is then added in the same manner to portion B and so on. The end elements and the shells of the mold are made of two parts assembled together by means of screw jaws as shown in Fig. 10, so as to permit of readily placing and removing them.

This method of manufacture is applicable in particular to screwed piles. It is also possible to build a pile that is sunk in the ground and then prolonged upwardly, with or without a change of section, owing to the use of suitable 5 molds, so as to obtain a pillar made of a single piece.

The second example relates to the production of large monolithic buildings of reinforced concrete, beams or arches for bridges, to which the 10 process according to my invention gives the advantage of an immediate striking of the center, even for considerable spans and extraordinarily high resistance to load. I may for instance build an arch made of elements of any section whatever, for instance of rectangular section. The mold shown in Fig. 17 consists of walls 90 and 91, assembled together and braced by means of bolts 92 passing through concrete tubes 93. It is caused to vibrate by the rotation of eccentric 20 masses, not shown in the drawings carried by shafts turning in bearings fixed to the wall 90 or to a filling hopper placed at a higher level, or through any other means. This mold consists of wall elements 90<sup>a</sup>, 90<sup>b</sup> which will adhere to the 25 concrete and are intended to remain fixed thereto; it further comprises cores 94 for the housing of connecting reinforcements, and other elastic cores 95 for the compression of the concrete, which may be flat as shown at 95<sup>a</sup>. The concrete 30 piece that is shown in the drawings can be developed by connecting it with contiguous elements added subsequently, in directions indicated by arrows F<sup>1</sup>, F<sup>2</sup> and F<sup>3</sup>, by making use of mold walls such as 101, 101<sup>a</sup>, 102, 102<sup>a</sup>, 103, 103<sup>a</sup> 35 shown in dotted lines, prolonging the mold 90, 91 and fixed either to the connecting elements 90<sup>a</sup>, 91<sup>a</sup>, or to the walls 90, 91, through any suitable means, eventually by means of a portion of the bolts 92 already utilized, after removal of the 40 portions of the molds such as 90<sup>b</sup>, 91<sup>b</sup>. The permanent connection between the successive concrete elements will be insured by holes provided in cores 94 and/or projecting reinforcements 96. The last mentioned reinforcements may be very 45 short and be prolonged by autogeneous welding, especially by utilizing the processes described in my French Patent No. 708,726, filed April 8, 1930. The concrete piece may also be prolonged in a direction at right angles to the plane of the 50 drawings, the connecting holes being then provided in cores disposed as at 95.

The last example shows that the advantages of my invention can be applied to constructions of any shape and size for which a high 55 resistance of the concrete and a quick hardening are desirable.

While I have described what I deem to be practical and efficient embodiments of my invention, it should be well understood that I do not 60 wish to be limited thereto, as there might be changes made in the arrangement, disposition and form of the parts without departing from the principle of my invention as comprehended within the scope of the appended claims.

What I claim is:

1. A process of manufacturing hollow concrete articles which comprises pouring wet concrete into a mold, fluidifying said concrete in said mold by rapid vibration and simultaneously subjecting 70 said liquid concrete to a pressure sufficiently low for permitting relative displacements of the particles of the concrete in the liquid mass, stopping the vibration when the concrete has become firm and finally subjecting said firm concrete in the 75

mold to a high pressure exerted from within the concrete mass.

2. A process of manufacturing hollow concrete articles which comprises pouring wet concrete into a mold and into a chamber communicating with the upper part of said mold, fluidifying said concrete in said mold and in said chamber by rapid vibration exerted on said mold and said chamber and simultaneously subjecting said liquid concrete to a pressure sufficiently low for permitting relative displacements of the particles of the concrete in the liquid mass, stopping the vibration when the concrete has become firm in the mold and finally subjecting said firm concrete in the mold to a high pressure exerted from within the concrete mass.

3. A process of manufacturing hollow concrete articles of elongated shape which comprises, pouring wet concrete into a mold of a shape corresponding to that of the article to be obtained and into a chamber communicating therewith and located above said mold, fluidifying said con-

crete by rapid vibration exerted on said chamber and said mold, whereby the liquid mass contained in the mold is subjected to a pressure sufficiently low for permitting relative displacements of the elements of the concrete under the effect of the vibrations, stopping the vibration when the concrete has become firm in said mold and finally reducing the volume of the concrete by deforming the mold in such manner as to reduce the area of the section thereof at right angles to its length, whereby the concrete in the mold is subjected to a high pressure.

4. A method of manufacturing articles of concrete which consists in pouring wet concrete into a mold, fluidifying said concrete by rapidly vibrating it and simultaneously subjecting said concrete to pressure, while allowing the excess of water to escape, whereby the mass of concrete is gradually compacted, then compressing said mass of concrete at high rate, and finally heating it.

EUGÈNE FREYSSINET.